

1

3,830,860

STABILIZATION OF NORBORNENES  
Tsuneyuki Nagase, Takatsuki, and Fujio Masuko,  
Ibaragi, Japan, assignors to Sumitomo Chemical Com-  
pany, Limited

No Drawing. Filed Jan. 26, 1973, Ser. No. 327,125  
Claims priority, application Japan, Jan. 27, 1972,  
47/10,383

Int. Cl. C07c 7/18  
U.S. Cl. 260—666.5

12 Claims 10

## ABSTRACT OF THE DISCLOSURE

A method for stabilization of norbornenes which comprises incorporating at least one phenol of either one of the formulae:



and



wherein X and X' are each alkylidene having 1 to 6 carbon atoms, cycloalkylidene having 3 to 6 carbon atoms, thio, sulfinyl or sulfonyl, R<sub>1</sub>, R<sub>2</sub>, R<sub>3</sub>, R<sub>4</sub>, R<sub>5</sub>, R<sub>6</sub>, R<sub>7</sub> and R<sub>8</sub> are each hydrogen, alkyl having 1 to 9 carbon atoms or cycloalkyl having 3 to 6 carbon atoms and R<sub>9</sub>, R<sub>10</sub>, R<sub>11</sub>, R<sub>12</sub>, R<sub>13</sub>, R<sub>14</sub> and R<sub>15</sub> are each hydrogen, alkyl having 1 to 9 carbon atoms or phenyl into a norbornene selected from the group consisting of alkenylnorbornenes alkylidenenorbornenes.

The present invention relates to a method for stabilization of norbornenes, particularly alkenylnorbornenes and alkylidenenorbornenes.

As is well known, norbornenes are very useful as one of the termonomers in the production of elastomers with ethylene and propylene (hereinafter referred to as "EPDM"). However, they are sensitive to air, metal oxides and the like and are apt to form rubbery materials on storage, whose presence is unfavorable, when the monomers are used for the production of terpolymer elastomers.

As the result of extensive studies, it has been found that some certain phenols are markedly effective for the stabilization of norbornenes.

According to the present invention, there is provided a method for stabilization of norbornenes which com-

2

prises incorporating at least one phenol of either one of the formulae:



wherein X and X' are each alkylidene having 1 to 6 carbon atoms, cycloalkylidene having 3 to 6 carbon atoms, thio, sulfinyl or sulfonyl, R<sub>1</sub>, R<sub>2</sub>, R<sub>3</sub>, R<sub>4</sub>, R<sub>5</sub>, R<sub>6</sub>, R<sub>7</sub> and R<sub>8</sub> are each hydrogen, alkyl having 1 to 9 carbon atoms or cycloalkyl having 3 to 6 carbon atoms and R<sub>9</sub>, R<sub>10</sub>, R<sub>11</sub>, R<sub>12</sub>, R<sub>13</sub>, R<sub>14</sub> and R<sub>15</sub> are each hydrogen, alkyl having 1 to 9 carbon atoms or phenyl into a norbornene selected from the group consisting of alkenylnorbornenes alkylidenenorbornenes.

As the norbornenes which can be stabilized by the present invention, there are exemplified alkenylnorbornenes of the formula:



40 [A]

wherein R<sub>16</sub>, R<sub>17</sub>, R<sub>18</sub> and R<sub>19</sub> are each hydrogen or alkyl having 1 to 6 carbon atoms and alkylidenenorbornenes of the formula:



45 [B]

50 where R<sub>20</sub>, R<sub>21</sub> and R<sub>22</sub> are each hydrogen or alkyl having 1 to 6 carbon atoms.

Specific examples of the alkenylnorbornenes [A] are as follows:

5-vinyl-2-norbornene,  
5-propenyl-2-norbornene,  
5-isopropenyl-2-norbornene,  
5-(2'-methylpropenyl)-2-norbornene,  
5-(1',2'-dimethyl-1'-propenyl)-2-norbornene,  
5-vinyl-6-methyl-2-norbornene, etc.

60 Specific examples of the alkylidenenorbornenes [B] are as follows:

5-methylene-2-norbornene,  
5-ethylidene-2-norbornene,  
5-isopropylidene-2-norbornene,  
5-ethylidene-6-methyl-2-norbornene,  
5-isopropylidene-6-methyl-2-norbornene, etc.

Among the phenols [I] and [II], particularly preferred are those wherein the substituents on the benzene rings represented by the symbols R<sub>1</sub> to R<sub>8</sub> are hydrogen, methyl, ethyl, propyl, isopropyl, sec.-butyl, t-butyl, t-octyl, sec.-nonyl, cyclohexyl and/or cyclohexylmethyl and the moiety

bridging two benzene rings represented by the symbols X or X' is methylene, ethylidene, isopropylidene, butylidene, cyclohexylidene, thio (—S—), sulfinyl (—SO—) or sulfonyl (—SO<sub>2</sub>—).

Specific examples of the phenols [I] and [II] are as follows:

4,4'-methylenebisphenol,  
4,4'-isopropylidenebisphenol,  
4,4'-cyclohexylidenebisphenol,  
4,4'-thiobisphenol,  
4,4'-methylenebis(2-t-butylphenol),  
4,4'-methylenebis(3-methyl-6-t-butylphenol),  
4,4'-isopropylidenebis(2-t-butylphenol),  
4,4'-butylidenebis(2-methylphenol),  
4,4'-thiobis(2-ethylphenol),  
4,4'-sulfonebis(2-cyclohexylphenol),  
4,4'-butylidenebis(3-methyl-6-t-butylphenol),  
4,4'-thiobis(3-methyl-6-t-butylphenol),  
4,4'-methylenebis(3,5-di-t-butylphenol),  
4,4'-methylenebis(3-methyl-5-t-butylphenol),  
2,2'-methylenebisphenol,  
2,2'-isopropylidenebisphenol,  
2,2'-thiobisphenol,  
2,2'-methylenebis(4-t-butylphenol),  
2,2'-thiobis(4-t-octylphenol),  
2,2'-methylene-bis(4-methyl-6-t-butylphenol),  
2,2'-thiobis(4-t-butyl-6-methylphenol),  
2,2'-methylenebis(4,6-di-t-butylphenol),  
2,2'-sulfonebis(4-t-butyl-6-methylphenol),  
2,2'-butylidenebis(4-t-butyl-6-methylphenol),  
etc.

Of the phenols [III], the preferred ones are those wherein the substituents on the naphthalene ring represented by the symbols R<sub>9</sub> to R<sub>15</sub> are methyl, ethyl, propyl, isopropyl, butyl, sec.-butyl, t-butyl, pentyl, isopentyl and/or phenyl.

Specific examples of the phenols [III] are as follows:

1-naphthol,  
2-methyl-1-naphthol,  
3-methyl-1-naphthol,  
4-methyl-1-naphthol,  
5-methyl-1-naphthol,  
7-methyl-1-naphthol,  
4-methyl-3-phenyl-1-naphthol,  
2-ethyl-1-naphthol,  
4-ethyl-1-naphthol,  
5-ethyl-4-methyl-1-naphthol,  
7-ethyl-4-methyl-1-naphthol,  
2,4-dimethyl-1-naphthol,  
2,7-dimethyl-1-naphthol,  
3,4-dimethyl-1-naphthol,  
5,7-dimethyl-1-naphthol,  
5,8-dimethyl-1-naphthol,  
2,4-diethyl-1-naphthol,  
2,4,6-trimethyl-1-naphthol,  
2,4,7-trimethyl-1-naphthol,  
3,4,6-trimethyl-1-naphthol,  
6-ethyl-2,4-dimethyl-1-naphthol,  
6-ethyl-3,4-dimethyl-1-naphthol,  
7-ethyl-3,4-dimethyl-1-naphthol,  
2-propyl-1-naphthol,  
4-propyl-1-naphthol,  
2-isopropyl-1-naphthol,  
5-isopropyl-3,8-dimethyl-1-naphthol,  
2-butyl-1-naphthol,  
4-butyl-1-naphthol,  
4-t-butyl-1-naphthol,  
2-sec.-butyl-1-naphthol,  
2-isopentyl-1-naphthol,  
2-phenyl-1-naphthol,  
4-phenyl-1-naphthol,  
2,3-diphenyl-1-naphthol,  
etc.

The concentration of the stabilizer, i.e. the phenol [I], [II] or [III], to be incorporated into the norbornene may be usually from about 20 p.p.m. to about 3000 p.p.m. or more. The preferred concentration is from 20 p.p.m. to 500 p.p.m. by weight, since at such concentrations the stabilizer need not be removed prior to use of the norbornene.

Practical and presently preferred embodiments of the present invention are illustratively shown in the following Examples wherein p.p.m. is by weight.

#### EXAMPLE 1

The desired quantity of stabilizer was added to freshly distilled 5-ethylidene-2-norbornene and charged in a glass ampoule. The ampoule without sealing was placed in an oil bath maintained at 54° C. After the elapse of a certain period of time, the ampoule was taken out from the oil bath and allowed to be cooled. 5-Ethylidene-2-norbornene was evaporated in vacuo, and the residual rubbery material was weighed. The results are shown in Table 1, compared with the results of the blank test without the addition of any stabilizer.

TABLE 1

| Stabilizer                                       | Concen-<br>tration<br>(p.p.m.) | Rubbery material (percent<br>by weight based on 5-<br>ethylidene-2-norbornene) |              |              |
|--------------------------------------------------|--------------------------------|--------------------------------------------------------------------------------|--------------|--------------|
|                                                  |                                | 184<br>hours                                                                   | 397<br>hours | 533<br>hours |
| None                                             |                                | 5.2170                                                                         | 11.8421      | 14.9704      |
| 4,4'-thiobis(3-methyl-6-t-<br>butylphenol)       | 254                            | 0.0209                                                                         | 0.1128       | 0.4629       |
| 2,2'-methylene-bis(4-methyl-<br>6-t-butylphenol) | 246                            | 0.0178                                                                         | 0.0138       | 0.1944       |

In the same manner as above, the stabilization effect of a conventional stabilizer, i.e. p-t-butylcatechol, on 5-ethylidene-2-norbornene was tested. The results are shown in Table A.

TABLE A

| Stabilizer        | Concen-<br>tration<br>(p.p.m.) | Rubbery material (percent<br>by weight based on 5-<br>ethylidene-2-norbornene) |                            |                          |
|-------------------|--------------------------------|--------------------------------------------------------------------------------|----------------------------|--------------------------|
|                   |                                | 184<br>hours                                                                   | 351<br>hours               | 639<br>hours             |
| p-t-Butylcatechol | { 345<br>100<br>50             | 0.077<br>0.081<br>4.024                                                        | 0.2768<br>3.3175<br>8.8175 | 0.471<br>5.997<br>11.489 |

In the same manner as in Example 1, the stabilization effect of the phenol as shown in Table 2 on 5-vinyl-2-norbornene was tested. The results are shown in Table 2, compared with that in case of the blank test.

TABLE 2

| Stabilizer                                            | Concen-<br>tration<br>(p.p.m.) | Rubbery material (percent by weight<br>based on 5-vinyl-2-norbornene) |              |              |              |
|-------------------------------------------------------|--------------------------------|-----------------------------------------------------------------------|--------------|--------------|--------------|
|                                                       |                                | 233<br>hours                                                          | 492<br>hours | 785<br>hours | 978<br>hours |
| None                                                  |                                | 2.6761                                                                | 6.2194       | 8.7498       | 13.3175      |
| 4,4'-thiobis(3-<br>methyl-6-t-butyl-<br>phenol)       | 266                            | 0.0603                                                                | 0.0890       | 0.1717       | 0.1945       |
| 2,2'-methylene-bis-<br>(4-methyl-6-t-<br>butylphenol) | 161                            | 0.0403                                                                | 0.0472       | 0.1565       | 0.1619       |

#### EXAMPLE 3

In the same manner as in Example 1, the stabilization effect of the phenol as shown in Table 3 or 5-isopropenyl-2-norbornene was tested. The results are shown in Table 3, compared with that in case of the blank test.

TABLE 3

| Stabilizer                                            | Concen-<br>tration<br>(p.p.m.) | Rubbery material (percent by weight<br>based on 5-isopropenyl-2-norbor-<br>nene) |              |              |              |
|-------------------------------------------------------|--------------------------------|----------------------------------------------------------------------------------|--------------|--------------|--------------|
|                                                       |                                | 245<br>hours                                                                     | 483<br>hours | 725<br>hours | 973<br>hours |
| None                                                  |                                | 2.752                                                                            | 6.013        | 9.731        | 15.425       |
| 4,4'-thiobis(3-<br>methyl-6-t-butyl-<br>phenyl)       | 235                            | 0.063                                                                            | 0.092        | 0.168        | 0.205        |
| 2,2'-methylene-bis-<br>(4-methyl-6-t-<br>butylphenol) | 198                            | 0.048                                                                            | 0.058        | 0.173        | 0.217        |

## EXAMPLE 4

In the same manner as in Example 1, the stabilization effect of the phenol as shown in Table 4 on 5-isopropylidene-2-norbornene was tested. The results are shown in Table 4, compared with that in case of the blank test.

TABLE 4

| Stabilizer                                            | Concen-<br>tration<br>(p.p.m.) | Rubbery material (percent by weight<br>based on 5-isopropylidene-2-norbor-<br>nene) |              |              |              |
|-------------------------------------------------------|--------------------------------|-------------------------------------------------------------------------------------|--------------|--------------|--------------|
|                                                       |                                | 179<br>hours                                                                        | 403<br>hours | 529<br>hours | 971<br>hours |
| None                                                  |                                | 4.071                                                                               | 9.753        | 12.692       | 16.352       |
| 4,4'-thiobis(3-<br>methyl-6-t-butyl-<br>phenyl)       | 238                            | 0.023                                                                               | 0.124        | 0.478        | 2.471        |
| 2,2'-methylene-bis-<br>(4-methyl-6-t-<br>butylphenol) | 225                            | 0.019                                                                               | 0.024        | 0.213        | 1.354        |

## EXAMPLE 5

In the same manner as in Example 1, the stabilization effect of the phenol as shown in Table 5 on 5-ethylidene-2-norbornene was tested. The results are shown in Table 5, compared with that in case of the blank test.

TABLE 5

| Stabilizer                                       | Concen-<br>tration<br>(p.p.m.) | Rubbery material (percent<br>by weight based on 5-<br>ethylidene-2-norbornene) |              |              |
|--------------------------------------------------|--------------------------------|--------------------------------------------------------------------------------|--------------|--------------|
|                                                  |                                | 191<br>hours                                                                   | 402<br>hours | 533<br>hours |
| None                                             |                                | 5.3243                                                                         | 12.0431      | 15.0025      |
| 2,2'-thiobis(4-t-butyl-6-<br>methylphenol)       | 238                            | 0.0213                                                                         | 0.1117       | 0.3419       |
| 4,4'-methylene-bis(3,5-di-t-<br>butylphenol)     | 213                            | 0.0227                                                                         | 0.0324       | 0.1869       |
| 4,4'-methylene-bis(3-methyl-<br>6-t-butylphenol) | 199                            | 0.0197                                                                         | 0.0248       | 0.3809       |
| 4,4'-isopropylidenebis(2-t-<br>butylphenol)      | 205                            | 0.0252                                                                         | 0.1043       | 0.2642       |

## EXAMPLE 6

In the same manner as in Example 1, the stabilization effect of the phenol as shown in Table 6 on 5-vinyl-2-norbornene was tested. The results are shown in Table 6, compared with that in case of the blank test.

TABLE 6

| Stabilizer                                       | Concen-<br>tration<br>(p.p.m.) | Rubbery material (percent<br>by weight based on 5-<br>vinyl-2-norbornene) |              |              |
|--------------------------------------------------|--------------------------------|---------------------------------------------------------------------------|--------------|--------------|
|                                                  |                                | 235<br>hours                                                              | 511<br>hours | 796<br>hours |
| None                                             |                                | 2.6873                                                                    | 6.3015       | 8.8102       |
| 2,2'-thiobis(4-t-butyl-6-<br>methylphenol)       | 185                            | 0.0613                                                                    | 0.0917       | 0.1843       |
| 4,4'-methylene-bis(3,5-di-t-<br>butylphenol)     | 203                            | 0.0598                                                                    | 0.0895       | 0.1739       |
| 4,4'-methylene-bis(3-methyl-<br>6-t-butylphenol) | 179                            | 0.0517                                                                    | 0.0749       | 0.1921       |
| 4,4'-isopropylidenebis(2-t-<br>butylphenol)      | 195                            | 0.0652                                                                    | 0.0825       | 0.1642       |

## EXAMPLE 7

In the same manner as in Example 1, the stabilization effect of the phenol as shown in Table 7 on 5-ethylidene-2-norbornene was tested. The results are shown in Table 7, compared with that in case of using 2-naphthol and that in case of the blank test.

TABLE 7

| Stabilizer | Concen-<br>tration<br>(p.p.m.) | Rubbery material (percent<br>by weight based on 5-<br>ethylidene-2-norbornene) |              |              |
|------------|--------------------------------|--------------------------------------------------------------------------------|--------------|--------------|
|            |                                | 266<br>hours                                                                   | 453<br>hours | 718<br>hours |
| None       |                                | 10.4933                                                                        | 13.6052      | 21.7987      |
| 1-naphthol | 482                            | 0.0701                                                                         | 0.1886       | 0.5505       |
| 2-naphthol | 301                            | 7.4271                                                                         | 15.3428      | 23.7229      |

## EXAMPLE 8

In the same manner as in Example 1, the stabilization effect of the phenol as shown in Table 8 on 5-vinyl-2-norbornene was tested. The results are shown in Table 8, compared with that in case of using 2-naphthol and that in case of the blank test.

TABLE 8

| Stabilizer | Concen-<br>tration<br>(p.p.m.) | Rubbery material (percent<br>by weight based on 5-vinyl-<br>2-norbornene) |              |              |
|------------|--------------------------------|---------------------------------------------------------------------------|--------------|--------------|
|            |                                | 247<br>hours                                                              | 479<br>hours | 791<br>hours |
| None       |                                | 2.7842                                                                    | 5.9834       | 8.9718       |
| 1-naphthol | 347                            | 0.0645                                                                    | 0.1731       | 0.2523       |
| 2-naphthol | 368                            | 1.9521                                                                    | 4.3718       | 7.5421       |

## EXAMPLE 9

In the same manner as in Example 1, the stabilization effect of the phenol as shown in Table 9 on 5-isopropenyl-2-norbornene was tested. The results are shown in Table 9, compared with that in case of using 2-naphthol and that in case of the blank test.

TABLE 9

| Stabilizer | Concen-<br>tration<br>(p.p.m.) | Rubbery material (percent<br>by weight based on 5-<br>isopropenyl-2-norbornene) |              |              |
|------------|--------------------------------|---------------------------------------------------------------------------------|--------------|--------------|
|            |                                | 243<br>hours                                                                    | 475<br>hours | 791<br>hours |
| None       |                                | 2.689                                                                           | 5.972        | 9.816        |
| 1-naphthol | 353                            | 0.075                                                                           | 0.143        | 0.306        |
| 2-naphthol | 371                            | 1.874                                                                           | 4.932        | 8.592        |

## EXAMPLE 10

In the same manner as in Example 1, the stabilization effect of the phenol as shown in Table 10 on 5-isopropylidene-2-norbornene was tested. The results are shown in Table 10, compared with that in case of using 2-naphthol and that in case of the blank test.

TABLE 10

| Stabilizer | Concen-<br>tration<br>(p.p.m.) | Rubbery material (percent<br>by weight based on 5-iso-<br>propylidene-2-norbornene) |              |              |
|------------|--------------------------------|-------------------------------------------------------------------------------------|--------------|--------------|
|            |                                | 193<br>hours                                                                        | 415<br>hours | 627<br>hours |
| None       |                                | 4.167                                                                               | 9.814        | 13.713       |
| 1-naphthol | 313                            | 0.072                                                                               | 0.182        | 0.563        |
| 2-naphthol | 341                            | 3.374                                                                               | 8.649        | 12.748       |

## EXAMPLE 11

In the same manner as in Example 1, the stabilization effect of the phenol as shown in Table 11 on 5-ethylidene-2-norbornene was tested. The results are shown in Table 11, compared with that in case of the blank test.

TABLE 11

| Stabilizer                          | Concen-<br>tration<br>(p.p.m.) | Rubbery material (percent<br>by weight based on 5-<br>ethylidene-2-norbornene) |              |              |
|-------------------------------------|--------------------------------|--------------------------------------------------------------------------------|--------------|--------------|
|                                     |                                | 273<br>hours                                                                   | 461<br>hours | 722<br>hours |
| None                                |                                | 10.5213                                                                        | 13.7145      | 21.8095      |
| 2-methyl-1-naphthol                 | 395                            | 0.0814                                                                         | 0.2135       | 0.6148       |
| 4-ethyl-1-naphthol                  | 418                            | 0.0903                                                                         | 0.2418       | 0.6719       |
| 6-ethyl-2,4-dimethyl-1-<br>naphthol | 453                            | 0.0857                                                                         | 0.3042       | 0.7143       |
| 4-butyl-1-naphthol                  | 393                            | 0.0932                                                                         | 0.3251       | 0.7521       |
| 4-phenyl-1-naphthol                 | 410                            | 0.0869                                                                         | 0.2981       | 0.6902       |

What is claimed is:

1. A method for stabilization of norbornenes which comprises incorporating at least one phenol of either one of the formulae:



and



wherein X and X' are each alkylidene having 1 to 6 carbon atoms, cycloalkylidene having 3 to 6 carbon atoms, thio, sulfinyl or sulfonyl, R<sub>1</sub>, R<sub>2</sub>, R<sub>3</sub>, R<sub>4</sub>, R<sub>5</sub>, R<sub>6</sub>, R<sub>7</sub> and R<sub>8</sub> are each hydrogen, alkyl having 1 to 9 carbon atoms or cycloalkyl having 3 to 6 carbon atoms and R<sub>9</sub>, R<sub>10</sub>, R<sub>11</sub>, R<sub>12</sub>, R<sub>13</sub>, R<sub>14</sub> and R<sub>15</sub> are each hydrogen, alkyl having 1 to 9 carbon atoms or phenyl into a norbornene selected from the group consisting of alkenylnorbornenes and alkylidenenorbornenes.

2. The method according to claim 1, wherein the alkenylnorbornenes are those of the formula:



wherein R<sub>16</sub>, R<sub>17</sub>, R<sub>18</sub> and R<sub>19</sub> are each hydrogen or alkyl having 1 to 6 carbon atoms.

3. The method according to claim 1, wherein the alkylidenenorbornenes are those of the formula:



wherein R<sub>20</sub>, R<sub>21</sub> and R<sub>22</sub> are each hydrogen or alkyl having 1 to 6 carbon atoms.

4. The method according to claim 1, wherein the concentration of the phenol to be incorporated is from 20 p.p.m. to 3000 p.p.m.

5. The method according to claim 4, wherein the concentration of the phenol to be incorporated is from 20 p.p.m. to 500 p.p.m.

6. The method according to claim 1, wherein the phenol is selected from the group consisting of

- 4,4'-methylenebisphenol,
- 4,4'-isopropylidenebisphenol,
- 4,4'-cyclohexylidenebisphenol,
- 4,4'-thiobisphenol,
- 4,4'-methylenbis(2-t-butylphenol),
- 4,4'-methylenbis(3-methyl-6-t-butylphenol),
- 4,4'-isopropylidenebis(2-t-butylphenol),
- 4,4'-butylidenebis(2-methylphenol),
- 4,4'-thiobis(2-ethylphenol),
- 4,4'-sulfonebis(2-cyclohexylphenol),
- 4,4'-butylidenebis(3-methyl-6-t-butylphenol),
- 4,4'-thiobis(3-methyl-6-t-butylphenol),
- 4,4'-methylenbis(3,5-di-t-butylphenol),

4,4'-methylenebis(3-methyl-5-t-butylphenol),

2,2'-methylenebisphenol,

2,2'-isopropylidenebisphenol,

2,2'-thiobisphenol,

2,2'-methylenebis(4-t-butylphenol),

2,2'-thiobis(4-t-octylphenol),

2,2'-methylenebis(4-methyl-6-t-butylphenol),

2,2'-thiobis(4-t-butyl-6-methylphenol),

2,2'-methylenebis(4,6-di-t-butylphenol),

2,2'-sulfonebis(4-t-butyl-6-methylphenol), and

2,2'-butylidenebis(4-t-butyl-6-methylphenol).

7. The method according to claim 1, wherein the phenol is selected from the group consisting of

1-naphthol,

2-methyl-1-naphthol,

3-methyl-1-naphthol,

4-methyl-1-naphthol,

5-methyl-1-naphthol,

7-methyl-1-naphthol,

4-methyl-3-phenyl-1-naphthol,

2-ethyl-1-naphthol,

4-ethyl-1-naphthol,

5-ethyl-4-methyl-1-naphthol,

7-ethyl-4-methyl-1-naphthol,

2,4-dimethyl-1-naphthol,

2,7-dimethyl-1-naphthol,

3,4-dimethyl-1-naphthol,

5,7-dimethyl-1-naphthol,

5,8-dimethyl-1-naphthol,

2,4-diethyl-1-naphthol,

2,4,6-trimethyl-1-naphthol,

2,4,7-trimethyl-1-naphthol,

3,4,6-trimethyl-1-naphthol,

6-ethyl-2,4-dimethyl-1-naphthol,

6-ethyl-3,4-dimethyl-1-naphthol,

7-ethyl-3,4-dimethyl-1-naphthol,

2-propyl-1-naphthol,

4-propyl-1-naphthol,

2-isopropyl-1-naphthol,

5-isopropyl-3,8-dimethyl-1-naphthol,

2-butyl-1-naphthol,

4-butyl-1-naphthol,

4-t-butyl-1-naphthol,

2-sec.-butyl-1-naphthol,

2-isopentyl-1-naphthol,

2-phenyl-1-naphthol,

4-phenyl-1-naphthol, and

2,3-diphenyl-1-naphthol.

8. A composition of matter comprising an alkenylnorbornene or an alkylidenenorbornene and a stabilizing amount of at least one phenol of either one of the formulae:



and



wherein X and X' are each alkylidene having 1 to 6 carbon atoms, cycloalkylidene having 3 to 6 carbon atoms,

thio, sulfinyl or sulfonyl, R<sub>1</sub>, R<sub>2</sub>, R<sub>3</sub>, R<sub>4</sub>, R<sub>5</sub>, R<sub>6</sub>, R<sub>7</sub> and R<sub>8</sub> are each hydrogen, alkyl having 1 to 9 carbon atoms or cycloalkyl having 3 to 6 carbon atoms and R<sub>9</sub>, R<sub>10</sub>, R<sub>11</sub>, R<sub>12</sub>, R<sub>13</sub>, R<sub>14</sub> and R<sub>15</sub> are each hydrogen, alkyl having 1 to 9 carbon atoms or phenyl.

9. A composition of matter in accordance with claim 8, wherein the alkenylnorbornene has the formula:



wherein R<sub>16</sub>, R<sub>17</sub>, R<sub>18</sub> and R<sub>19</sub> are each hydrogen or alkyl having 1 to 6 carbon atoms.

10. A composition of matter in accordance with claim 8, wherein the alkylidenenorbornene has the formula:



5

wherein R<sub>20</sub>, R<sub>21</sub> and R<sub>22</sub> are each hydrogen or alkyl having 1 to 6 carbon atoms.

11. A composition of matter in accordance with claim 8, wherein the stabilizing amount of phenol in said composition is from 20 p.p.m. to 3000 p.p.m.

12. A composition of matter in accordance with claim 8, wherein the stabilizing amount of phenol in said composition is from 20 p.p.m. to 500 p.p.m.

10

## References Cited

## UNITED STATES PATENTS

|           |         |                |           |
|-----------|---------|----------------|-----------|
| 3,409,683 | 11/1968 | Britton et al. | 260—666.5 |
| 3,487,044 | 12/1969 | Tholstrup      | 260—45.85 |
| 3,527,822 | 9/1970  | Benson         | 260—666.5 |
| 3,660,352 | 5/1972  | Song           | 260—666.5 |

DELBERT E. GANTZ, Primary Examiner

J. M. NELSON, Assistant Examiner

20

U.S. Cl. X.R.

260—666 A